

F. W. TULLY.

RUG, MAT, OR OTHER COVERING, AND METHOD OF MAKING THE SAME.  
APPLICATION FILED JAN. 19, 1916.

1,223,538.

Patented Apr. 24, 1917.

Fig. 5.



Fig. 1.



Fig. 4.



Fig. 2.



Fig. 3.



Inventor:

Francis W. Tully  
by *Thomas Edwards & Cushman*  
his Attorneys.

# UNITED STATES PATENT OFFICE.

FRANCIS W. TULLY, OF BROOKLINE, MASSACHUSETTS.

## RUG, MAT, OR OTHER COVERING AND METHOD OF MAKING THE SAME.

1,223,538.

Specification of Letters Patent.

Patented Apr. 24, 1917.

Application filed January 19, 1916. Serial No. 73,045.

*To all whom it may concern:*

Be it known that I, FRANCIS W. TULLY, a citizen of the United States, and resident of Brookline, in the county of Norfolk and State of Massachusetts, have invented new and useful Improvements in Rugs, Mats, or other Coverings and Methods of Making the Same, of which the following is a specification.

10 This invention relates to rugs, mats, carpets and other coverings, one object of my invention being to prevent slippage of such an article when placed on a slippery surface such as a polished floor, as well as to provide means whereby the rugs, etc., are made to lie flat upon the floor, and to resist their tendency to wrinkle or curl.

Such coverings in use, but especially mats and rugs intended for floor-coverings, are 20 rendered of less than their full utility when fastened to the floor or other surface, and are the frequent cause of accidents to persons stepping on them when not fastened.

Various methods and devices have heretofore been resorted to for preventing slippage, but all such devices of which I am aware have defects fully accounting for the failure of any general use of such devices. Metal devices attached to the rug for engagement with the floor are injurious to the floor 30 when not intended for a definite place on the floor, and when intended for a definite place limit the usefulness of the rug or mat except in that place, and prevent random placing of 35 the rug so as to avoid destructive wear at parts only thereof. The metal fastening itself, of whatever form, makes a projection under the rug above which destructive wear takes place rapidly. Rubber patches, or

40 patches of rubber cloth, sometimes fastened on the under surface of the rug, while free from objectionable damage to the floor and permitting the rug to be moved about, invariably present ridges or projections above 45 which the surface of the rug wears off in use, besides being ineffective unless so large and frequent as to be too expensive for ordinary use. I attribute the lack of effect of rubber-cloth and the like to the insufficiently yielding and insufficiently sticky surface of 50 such materials, which will not hold against a sharp lateral strain unless subjected to considerable pressure, as by being stepped upon directly over the patch by a person 55 walking on the rug. The mere weight of the

rug is usually insufficient to cause such patches to adhere and become effective.

One object of my invention is to provide an attachment for such coverings which will be free from the disadvantages mentioned. 60 Another object is to provide such a covering with a readily attached frictional holding surface which will not materially project a part of the covering to which it is applied above the remainder thereof, so as to cause local wear, and which shall be adapted for frictionally holding rugs of a soft texture, such as oriental or tufted pile rugs of various or irregular patterns or structures of fabric. Another object is to provide a structure adapted to adhere to a support by the mere weight of the fabric to which it is applied, and other objects are to provide an addition to existing fabrics for the above and other purposes adapted to be applied 70 rapidly and with economy of time and materials.

In the accompanying drawings,

Figure 1 is a schematic section through a fabric illustrating one form of my invention; 80

Fig. 2 is an under plan view of a rug comprising one application of my invention;

Fig. 3 is an under plan view of an oriental rug illustrating another application 85 thereof;

Fig. 4 is a schematic section of an Axminster carpet fabric illustrating another embodiment of my invention; and

Fig. 5 shows my invention in connection 90 with a fabric of the ingrain type.

Referring now to Fig. 1, the fabric therein shown comprises warps 1 and a knotted weft pile 2, being typical of oriental and other tufted pile fabrics, wherein the soft 95 yarn of the ornamental pile surface reaches the back and forms the surface of the fabric which rests upon the floor or other support therefor. Fabrics of other types, such as Axminster fabrics, Fig. 4, in which stuffer 100 yarns are used to give body are sometimes treated with a glue or starch size or other stiffening material, but fabrics of the class above mentioned are not customarily so treated.

For the purposes of my present invention, I first apply a coating adapted to become adherent to or incorporated by a shallow penetration only with all or portions only 105 of the back face of the fabric. As illus-

trated in Fig. 2, lines 3 forming closed rectangular figures, for instance, may be applied to the back of the rug. These lines are formed by padding, stenciling or painting with a brush, or by other suitable means of applying the sizing material, the result being an adherent, non-absorbent coating 4, as illustrated in Fig. 1, at the places where the coating 4 is applied.

10 In some cases and in the treatment of some fabrics I may apply the coating 4 continuously upon the back surface of the rug or other fabric.

One practicable coating comprises an 15 aqueous solution of glue sufficiently stiff to prevent much penetration of the cloth to which it is applied, but I prefer a relatively stiff solution of rubber in naphtha or other volatile solvent, sparingly applied, or an 20 alcoholic or other non-aqueous solution of certain gums or other colloids such as pine resin, tragacanth or other commercial gums. One purpose of the coating 4 is to fill the 25 interstices of the back face of the fabric to prevent absorption into the fabric of a subsequent sticky coating, which purpose will be carried out when the application is of any composition of matter furnishing a coat rendering the back of the fabric impermeable to another superposed coating after the 30 first or sizing coating 4 is dried or set. I may, for instance, make a coating 4 of an inert substance such as celluloid, using a solution in acetone, or employ any other suitable 35 varnish or plastic to form a layer resisting penetration into the fabric of the rug of a liquid or semi-liquid adhesive coating to be applied over the coating 4, continuously or at places only, to enable the rug 40 or other fabric to adhere to the floor or other support. I wish to emphasize the importance of the coating 4, since I have found that without such an application it is difficult and commercially impracticable to apply a sticky coating in sufficient volume for 45 my purpose without causing it to penetrate to and spoil the face of the fabric, or to be wastefully absorbed, or to affect the texture of the fabric detrimentally.

50 Rugs of the type mentioned are improved as articles of use and wear by the application of such a coating 4, which has the effect of preventing longitudinal or transverse elasticity of the rug, without materially 55 affecting its flexibility.

I now apply upon the sized area in a fluid or semi-fluid state a composition of matter suitable to form a coating 5 adapted to adhere to a polished floor or other supporting 60 surface. As one instance only, I find that a solution of crude rubber in naphtha is well adapted to my said purposes. The sticky substance so dissolved may, however, comprise any suitable rubber compound, oxidized oil or any viscolized or partially vul-

canized gummy substance having the quality of adhesion without complete attachment to polished surfaces. The solvent mentioned may be replaced by other suitable solvents such as carbon tetrachlorid or, in the case of 70 crude rubber, and preferably, a solvent comprising two parts of naphtha to one part of carbon tetrachlorid may be employed, the rubber being dissolved in the solvent until the solution is in the condition of free-flowing paint.

In some cases I find that the objects of my invention may be attained by painting a 75 coating 4 of the adhesive solution above mentioned on the back of the rug or other 80 fabric without previous treatment, the procedure in that case being first to stretch the rug or other fabric, and then to give it a light, continuous coat of the adhesive substance, which is permitted to dry while the 85 rug remains stretched. A second coat 5 suitable to adhere to the floor of the adhesive substance may now be applied in larger quantities without danger of penetrating the fabric of the rug so completely 90 as to affect its wear surface. The second coat may be applied continuously or, if desired, may be applied in a pattern such as that shown in Fig. 2.

In some cases I prefer, as illustrated in 95 Fig. 3, to apply the coatings 4 and 5, or the coating 5 only on the elements of the pattern woven in the rug, for instance, if the rug is an oriental rug, as suggested in the figure, the darker units 6 of the pattern 100 at the back of the rug may be selected for the application of the sizing coating 4 and the adhesive coating 5.

When the rug is the type of rug permitting 105 cleansing by washing, such as an oriental rug, I prefer for both coatings a solution of rubber or other gum in a volatile non-aqueous solvent, a rug so treated being capable of being washed repeatedly without removing the adhesive coatings or 110 damaging their quality of adhesion.

When a rug so treated is placed on the 115 floor, adhesion by its own weight is sufficient to prevent slippage when the rug is stepped on. Other advantages follow, for instance the prevention of curling of the corners, the coating having a marked effect to prevent folds or curling at the edges. If desired, lines of sewing stitches 7 lying transverse to the edges may be applied at the corners of the rug prior to coating with the sizing or the adhesive coatings 4 and 5, for the complete prevention of curling at the corners.

When the coating 5 has been applied, the 125 solvent is driven off by exposure to dry air or to heat, or both. The residual coating 5 retains indefinitely the quality of adhesion to surfaces such as glass, marble, tiling, and polished or varnished wood under very 130

slight pressure, such as the weight of the fabric, and I find rugs and mats made by the above described method to be safe against slipping in situations in which any 5 of the structures of the present art of which I am aware, except positive fastening means, are liable to slip.

What I claim is:

1. A rug or mat having on one face a sizing coating and a superposed adherent plastic coating of an adhesive substance. 10

2. A rug or mat having on one face an adherent coating incorporated by shallow penetration only with one face thereof, and an adhesive coating superposed upon and plastically adherent to said first-mentioned coating. 15

3. A rug or mat having on one face an applied pattern or figure comprising areas of a sizing coating and a plastically adherent superposed adhesive substance. 20

4. A rug or mat having on one face a coating comprised of an adherent substance insoluble in water, and an adhesive coating 25 plastically applied to and superposed upon said adherent coating.

5. A rug or mat having an adherent sizing coating on one face thereof of a substance insoluble in water, and an adhesive 30 coating of a rubber compound remaining sticky when dry.

6. A rug or mat having on the back face thereof an adherent sizing coating and an adhesive coating adapted to cling to a polished floor or other support, and composed 35 of a gummy substance remaining as a resin-

due after the evaporation of a volatile solvent.

7. The method of rendering rugs, mats or other coverings adherent with respect to a 40 supporting surface, comprising first coating the back of a suitable textile fabric with a sizing coating of a consistency adapted to adhere without penetrating to the front surface of said fabric, drying said coating, and 45 then applying in a plastic condition a coating of a sticky substance dissolved in a volatile solvent.

8. The method of treating rugs, mats or other coverings to cause them to be adapted 50 to cling to a supporting surface, comprising first stretching a suitable textile fabric, then coating the back of said fabric with a sizing coating of a consistency adapted to adhere without penetrating to the front surface of 55 said fabric, drying said coating while the fabric is stretched, and then applying in a plastic condition a coating of an adhesive containing rubber dissolved in a volatile solvent. 60

9. The method of treating rugs, mats or other coverings to cause them to be adapted to cling to their supporting surface, comprising first treating the back of a suitable fabric to render it impermeable, then applying in a plastic condition an adherent coating of a sticky substance dissolved in a volatile solvent, and then evaporating the solvent. 65

Signed by me at Boston, Massachusetts this seventeenth day of January 1916.

FRANCIS W. TULLY.